

## 1

3,397,127

**METHOD AND BATH FOR ELECTRO-  
PLATING GOLD**

Eldridge K. Camp, Watertown, Conn., assignor to American Chemical & Refining Company, Incorporated, Waterbury, Conn., a corporation of Connecticut  
No Drawing. Filed Apr. 12, 1965, Ser. No. 447,536  
13 Claims. (Cl. 204—46)

**ABSTRACT OF THE DISCLOSURE**

There is disclosed a method of plating gold wherein a soluble gold cyanide complex salt is dissolved in water and the resultant solution acidified to a pH of about 2.0—5.0 to expel substantially all free cyanide therefrom. The pH of the solution is thereafter raised to a value of about 6.1—10.5 at which the plating operation is conducted with an electroplating current to produce gold plated articles having uniform surfaces with a low edge to center ratio.

The present invention relates to a novel bath and method for plating high-purity gold.

Generally, the more commonly employed baths for the electroplating of gold utilize cyanide ion in excess of the amount of gold present. Because of the noxious nature of hydrogen cyanide, such baths customarily are employed at a highly alkaline pH with limitations as to application and hazards to personnel. There have been proposals for cyanide-free baths set forth in Smith United States Patent 3,057,789 and Ehrhardt French Patent 1,265,517. These patents and others have proposed baths which might be operated at acid or nearly neutral pH including Volk United States Patent 2,812,299. However, one of the most common shortcomings of various baths for electroplating gold has been a tendency for a much greater deposit thickness adjacent the edges of the workpiece than at the center with resultant increased cost to achieve the minimum thickness.

It is an object of the present invention to provide a novel bath and method for the plating of gold which will yield a low edge to center ratio in the thickness of the plated metal with readily controllable deposit thickness.

It is also an object of the present invention to provide such a bath and method having extremely high covering power and relatively long life and which is relatively economical in operation.

Another object is to provide such a bath and method which yield an ultrahigh purity deposit of gold having high ductility and a desirable controlled appearance.

Still another object is to provide a plated article having a deposit of gold thereon with a low edge to center ratio and desirable controlled appearance and high ductility.

It has now been found that the foregoing and related objects can be readily attained by a method in which a soluble gold cyanide complex salt is dissolved in water to provide a solution which is then acidified to a pH of about 2.0—5.0 to drive off some cyanide therefrom. The pH of the solution is then raised to about 6.1—10.5 for the plating operation which generally will be electroplating although the bath may also be employed for chemical plating.

By use of the present invention it has been found possible to consistently obtain gold deposits of extremely high purity having an edge to center ratio of less than 1.4:1 and generally less than 1.3:1 and even below 1.2:1. The deposits have a desirable light metallic yellow appearance and a reflection which may vary from lustrous to satin. An unsupported electroplate has been bent upon itself without evidence of cracking and the deposit has been

## 2

found to have a Vickers hardness within the range of 50.0 to 75.0 kilograms per square millimeter at a 50 gram load. The bath may be operated at a wide range of current density varying from 0—16.5 amperes per square decimeter with a relatively high degree of current efficiency.

The theory of operation of the present invention is not fully understood. Many commercial gold cyanide complex salts contain cyanide ion in excess of two mols of cyanide to every mol of gold. Even with those salts which are of high purity so as to have the proper molar equivalents, the present invention has been found applicable in that some portion of the combined cyanide appears to be eliminated in the form of hydrogen cyanide while still retaining some amount of the gold as the soluble gold cyanide complex salt. In subsequent operation of the bath even at temperatures at or near boiling, the fact that there is minimal evolution of hydrogen cyanide and very little build up of carbonates in the bath is quite significant. It is believed that the cyanide retained in the acidified and subsequently neutralized bath is sufficient to produce enhanced operation while at the same time avoiding the development of any excess cyanide ion such as might produce deleterious effects.

The soluble gold cyanide complex salts employed in accordance with the present invention should not introduce any interfering cations. Generally the salts which fall within this category may be classified as alkali metal and ammonium gold cyanide. Potassium gold cyanide and sodium gold cyanide have proven particularly effective and are readily available. The gold content may range from 4.0 to 500.0 grams per liter and preferably 6.0 to 15.0 grams per liter.

The solution of the complex salts may be acidified to a pH of 5.0 or below by use of an acid or acid salt which will not introduce an interfering anion or cation. Phosphoric acid, sulfuric acid, sulfamic acid, hydrochloric acid, tartaric acid, acetic acid, nitric acid and citric acid or the acid salts thereof, have all been employed with varying degrees of effectiveness. Phosphoric acid and its acid salts have been found preferable for operation in the present invention although acetic acid and tartaric acid also have produced desirable results.

Although the expelling of the cyanide ion will occur slowly at ambient temperatures particularly at a low pH, generally it is desirable to accelerate the procedure by use of elevated temperatures and agitation. For example, at a pH of approximately 4.0, the acidified solution may be merely brought to a boil rapidly and cooled or it may be held at a temperature of approximately 77° C. for a period of up to one hour. The conditions employed should not destroy all the gold cyanide complex salt present in the solution.

After the expulsion of the cyanide ion, the pH of the bath is then elevated to the range of 6.1—10.5 and preferably about 6.3—7.3 for optimum operation for most applications. A non-interfering base such as ammonium or the alkali metal hydroxides may be employed for this purpose or suitable basic salts may also be used such as diammonium phosphate, disodium phosphate, etc.

The agents used to acidify and neutralize the solution should provide a current-carrying radical or anion in the amount of at least 10 grams per liter and preferably 15 grams per liter, and up to saturation. Although various anions have been tested and utilized with varying degrees of effectiveness as set forth herebefore, the most desirable operation has been obtained by use of phosphates as the acidifying and neutralizing agents, although a highly desirable degree of operation has been observed with respect to tartrates and acetates. The data concerning the efficacy of the several anions is set forth in Table 1 below.



cyanide, the pH was adjusted to above 6.1 with ammonium hydroxide alone in Baths 1, 4, 6 and 7; by sodium hydroxide and ammonium hydroxide in Baths 2 and 3; and by potassium hydroxide in Bath 5. Additional salts were added in some instances to provide sufficient current-carrying anion. The several substances added to the solution of potassium gold cyanide are set forth in Table 3 above. Test panels were prepared by plating at a temperature of about 67° C., the current density, time, deposit thickness, and pH of the several baths being shown in Table 1 hereinbefore for three separate test panels prepared in each bath. The test panels were nickel panels one-half inch by two inches and five mils in thickness. The baths were operated at a temperature of about 69° C.

In all instances, a satisfactory gold deposit was obtained but the color of the panels produced by the sulfamate and chloride baths was a little orange-like. As can be seen, the nitrate and citrate baths were low in current efficiency.

#### Example 4

A bath was prepared by dissolving ten grams per liter of water of potassium gold cyanide and acidifying the solution with 50 grams per liter of ammonium dihydrogen phosphate. After heating the bath to expel cyanide therefrom, the bath was neutralized to a pH of about 6.5 by addition of 5 grams per liter of sodium hydroxide and adjustment to the end point with ammonium hydroxide.

A nickel panel two inches by one-half inch and 5 mils in thickness was immersed therein at a temperature of 77° C. for a period of six minutes with no current applied to the bath. Upon removal the panel was observed to have a bright gold deposit of about three microinches in thickness.

#### Example 5

Potassium gold cyanide was dissolved in water to provide 400 grams per liter and the solution was then acidified by the addition thereto of 48 grams per liter of ammonium dihydrogen phosphate. After heating to drive off cyanide, 84 grams per liter of diammonium phosphate was added thereto and the pH was adjusted to 6.3 with ammonium hydroxide.

A graphite cathode was immersed therein and the bath was operated at a temperature of 71° C. A current of 4.40 amperes per square decimeter was applied between the anode and cathode. The resultant metallic deposit had a satin, highly pleasing appearance.

Thus it can be seen from the foregoing detailed specification and example that the present invention provides a novel bath and method for the plating of gold which yields a low edge to center ratio in the plated metal and facile control of the thickness of the deposit. The bath is relatively economical in operation and has extremely high covering power and long life. The gold deposit produced thereby has high ductility, a desirable controlled appearance and a satin finish particularly in the heavier deposits which are possible herewith. Electroforms produced therefrom can tolerate temperatures approaching the melting point without blistering, distortion or discoloration.

Having thus described the invention, I claim:

1. In the method of electroplating gold, the steps comprising dissolving in water a complex gold salt selected from the group consisting of ammonium gold cyanide and alkali metal gold cyanide in an amount sufficient to provide 4.0 to 500 grams per liter of gold; acidifying the resultant solution with an acid agent to a pH of about 2.0-5.0; heating the acidified solution to drive off substantially all free cyanide therefrom; and thereafter adding a neutralizing agent to raise the pH of the solution to about 6.1 to 10.5, the acidifying and neutralizing agents providing a current-carrying radical in the amount of about 15 grams per liter to saturation.

2. The method of claim 1 wherein said acidifying agent is a phosphate compound.

3. The method of claim 1 wherein the pH of the neutralized solution is about 6.3 to 7.3.

4. In the method of electroplating gold, the steps comprising dissolving in water a soluble gold cyanide complex salt selected from the group consisting of ammonium gold cyanide and alkali metal gold cyanides in an amount sufficient to provide 4.0 to 500.0 grams per liter of gold; acidifying the resultant solution to a pH of about 2.0-5.0 and expelling substantially all free cyanide therefrom; thereafter raising the pH of the resultant solution to about 6.1-10.5; placing in said solution a cathode and an anode; and passing current between said anode and cathode to plate gold upon said cathode to the desired thickness at the center thereof, the plated gold having an edge to center ratio of less than 1.4:1.

5. The method in accordance with claim 4 wherein said solution is raised to a pH of 6.3 to 7.3.

6. In the method of electroplating gold, the steps comprising dissolving in water a complex gold salt selected from the group consisting of ammonium gold cyanide and alkali metal gold cyanide in an amount sufficient to provide 4.0 to 500.0 grams per liter of gold; acidifying the resultant solution with an acid agent to a pH of about 2.0-5.0; heating the acidified solution to drive off substantially all free cyanide therefrom; thereafter adding a neutralizing agent to raise the pH of the solution to about 6.1 to 10.5, the acidifying and neutralizing agents providing a current-carrying radical in the amount of about 15 grams per liter to saturation; placing in said solution a cathode and an anode; and passing a current of about 0.1-0.8 ampere per square decimeter between said anode and cathode to plate gold upon said cathode to the desired thickness at the center thereof, the plated gold having an edge to center ratio of less than 1.4:1.

7. The method of claim 6 wherein said acidifying agent is a phosphate compound.

8. The method of claim 6 wherein the pH of the neutralized solution is about 6.3 to 7.3.

9. The method of claim 6 wherein said edge to center ratio is less than 1.25:1.

10. A bath for electroplating gold comprising an aqueous solution containing a gold cyanide complex salt selected from the group consisting of ammonium gold cyanide and alkali metal gold cyanides and a current-carrying radical in the amount of 15 grams per liter to saturation, said solution containing 4.0 to 500.0 grams per liter of gold and having a pH of about 6.1 to 10.5, said solution being substantially free from free cyanide ion and having been acidified initially to a pH of about 2.0-5.0 and heated to drive off substantially all free cyanide.

11. The bath of claim 10 wherein said solution has a pH of 6.3 to 7.3.

12. The bath of claim 10 wherein said current-carrying radical is a phosphate ion.

13. A bath for plating gold comprising an aqueous solution containing a gold cyanide complex salt selected from the group consisting of ammonium gold cyanide and alkali metal gold cyanides and phosphate ion in the amount of 15 grams per liter to saturation, said solution containing 4.0 to 500.0 grams per liter of gold having a pH of about 6.3 to 7.3, said solution being substantially free from free cyanide ion and having been acidified initially to a pH of about 2.0 to 5.0 and heated to expel substantially all free cyanide therefrom.

#### References Cited

#### UNITED STATES PATENTS

|           |        |                      |           |
|-----------|--------|----------------------|-----------|
| 2,905,601 | 9/1959 | Rinker et al. -----  | 204-46 XR |
| 2,967,135 | 1/1961 | Ostrow et al. -----  | 204-46 XR |
| 2,978,390 | 4/1961 | Atwater et al. ----- | 204-46    |
| 3,123,484 | 3/1964 | Pokras et al. -----  | 106-1     |
| 3,303,111 | 2/1967 | Peach -----          | 204-38    |

JOHN H. MACK, Primary Examiner.

75 G. KAPLAN, Assistant Examiner.